

## UNITED STATES PATENT OFFICE

JOSEF TALALAY AND WILHELM HOLZBERG, OF BERLIN, GERMANY, ASSIGNEES TO  
FELIX PEEFER, OF NEW YORK, N. Y.

## CLEANING COMPOUND

No Drawing.

Application filed August 18, 1925. Serial No. 51,044.

Our invention relates to cleaning compounds, and more particularly to compounds of a comparatively consistent character which may be moulded or pressed into tablets, rods or the like and are particularly suitable for cleaning hard objects such as steel stamps, type writing machines, etc., and it is an object of our invention to provide a compound of the kind described which does not "age", that is, does not lose its plasticity and dirt-absorbing qualities in time. To this end, we mix with the compound substances which are suitable for maintaining it in its plastic condition, and substances rich in resin, and so obtain a compound of practically unlimited life.

Heretofore, objects of the kind referred to were either cleaned with petrol applied by a brush, or with a pasty substance. The former method is tedious and dirty, and the pastes as heretofore made involved the drawbacks of rapid "aging" so that they had to be used within a short period from their manufacture as else they would lose their plasticity and their dirt-absorbing qualities, the latter due to volatilization of their resinous constituents.

These drawbacks are overcome in accordance with our invention by admixing to said compounds either mineral oils or non-drying or semi-drying vegetable oils such as rape-seed oil, and rubber varieties rich in resin, such as guayule, agra flakes, ficus, etc., the other constituents of the compound being, for instance, factice, brown or white, chalk, heavy spar (sulfate of barium), lithopone, lime, infusorial earth, a colouring agent (ultramarine blue, cobalt blue, soot black, iron oxide, typoforod, cinnabar), powdered marble, zinc white, kaolin, and combinations thereof.

The resin contained in the rubber can be partly or completely substituted by gutta percha resin, dead borneo (a resinous crude rubber) etc., and suitable regenerates may be used instead of rubber.

Preferably, the oil is heated, the resinous rubber is dissolved in the oil so as to prevent hardening of the resin at a later period, thus

increasing the life of the compound and its dirt-absorbing qualities.

The percentage of the constituents may vary. The compositions of four suitable compounds are given below in percentages by weight:

## No. I

| Substance              | Percentage by weight |      |
|------------------------|----------------------|------|
| Rubber (rich in resin) | 12.65                | 60   |
| Brown factice          | 12.9                 |      |
| Chalk                  | 23.6                 |      |
| Heavy spar             | 18.5                 |      |
| Kaolin                 | 3.                   | 65   |
| Powdered marble        | 2.1                  |      |
| Lithopone              | 13.9                 |      |
| Lime                   | 1.45                 |      |
| Ultramarine blue       | .85                  |      |
| Mineral oil            | 7.05                 | 70   |
|                        |                      | 100. |

## No. II

| Substance                  | Percentage by weight |      |
|----------------------------|----------------------|------|
| Rubber (15 per cent resin) | 9.43                 |      |
| Regenerate, clear          | 25.16                |      |
| Factice, brown             | 6.29                 |      |
| Factice, light             | 6.29                 | 80   |
| Lithopone                  | 25.16                |      |
| Heavy spar                 | 18.87                |      |
| Mineral oil                | 7.86                 |      |
| Ultramarine blue           | .94                  |      |
|                            |                      | 85   |
|                            |                      | 100. |

## No. III

| Substance                          | Percentage by weight |      |
|------------------------------------|----------------------|------|
| Rubber II (5 per cent resin)       | 9.43                 |      |
| Factice, brown                     | 12.58                |      |
| Lithopone                          | 25.16                |      |
| Heavy spar                         | 18.87                |      |
| Mineral oil or rape seed oil       | 7.86                 | 95   |
| Ultramarine blue or iron oxide     | .94                  |      |
| Powdered marble                    | 22.                  |      |
| Resin, dead borneo or gutta percha | 3.16                 |      |
|                                    |                      | 100. |

| Substance           | No. IV | Percentage<br>by weight | heavy mineral filler, lithopone, and a mineral oil.                                                                                                                                               |
|---------------------|--------|-------------------------|---------------------------------------------------------------------------------------------------------------------------------------------------------------------------------------------------|
| Rubber II           |        | 10                      | 4. A type cleaner comprising a plastic cake formed of a mechanical mixture of powdered calcium carbonate, plastic rubber containing resin, factice, a heavy mineral filler, and a mineral oil. 70 |
| 5 Guayule           |        | 16                      |                                                                                                                                                                                                   |
| Factice, brown      |        | 28                      |                                                                                                                                                                                                   |
| Factice, white      |        | 10                      |                                                                                                                                                                                                   |
| Mineral oil         |        | 1                       |                                                                                                                                                                                                   |
| Zinc white          |        | 6                       |                                                                                                                                                                                                   |
| 10 Kaolin           |        | 8                       |                                                                                                                                                                                                   |
| Heavy spar          |        | 6                       |                                                                                                                                                                                                   |
| Chalk               |        | 4                       |                                                                                                                                                                                                   |
| Precipitated silica |        | 4                       |                                                                                                                                                                                                   |
| Lithopone           |        | 6                       |                                                                                                                                                                                                   |
| 15 Ultramarine blue |        | 1                       |                                                                                                                                                                                                   |
|                     |        | 100                     |                                                                                                                                                                                                   |

Factice brown consists of plant oils that are mixed with sulphur and boiled and admixtures of mineral oil and fillers such as chalk, feldspar and the like can likewise be made.

Factice light also consists of plant oils, chiefly rapeseed oil, mixed with carbon disulphide (2-8%) or with sulphur chloride. The brown factice is produced from the plant oils, such as linseed, rapeseed, castor and the like by treatment with heat whereas in forming white factice the oils are treated while cold.

Regenerate clear is regenerated rubber that, when ground up, is freed from free sulphur.

The mineral oil used has the ordinary properties, and an average boiling point of 350° C.

The constituents are mixed and kneaded into a plastic sticky consistence, and the compound may then be moulded into tablets or sticks. When such a stick or the like is moved along the parts to be cleaned under pressure, the dirt adheres to the stick and the parts become bright or clean instantly. The stick may be used repeatedly, being simply remoulded after having been used.

Any colouring agent may be added to the compound. Its colour may be the same as that of the dirt to be removed or some other colour which differs widely from that of the dirt. In the latter case, the colour of the stick indicates its condition, as its original colour will gradually be effaced by that of the dirt.

We claim:

1. A composition of matter for cleaning type, containing a base of powdered inert mineral substance, plastic rubber, factice, a heavy mineral filler, and a mineral oil.
2. A type cleaner comprising a plastic cake formed of a mechanical mixture of powdered calcium carbonate, plastic rubber, factice, a heavy mineral filler, and a mineral oil.
3. A type cleaner comprising a plastic cake formed of a mechanical mixture of powdered calcium carbonate, plastic rubber, factice, a

heavy mineral filler, lithopone, and a mineral oil.

5. A type cleaner comprising a plastic cake formed of a mechanical mixture of powdered calcium carbonate, plastic rubber containing resin, factice, a heavy mineral filler, and a mineral oil. 75

6. A type cleaner comprising a plastic cake containing between 9% and 13% rubber, containing at least 5% of its weight of resin; substantially 12% of factice; substantially 18% heavy spar; and substantially 7% mineral oil and over 13% of lithopone. 80

7. A type cleaner comprising a plastic cake containing a base of calcium carbonate at least 22%; between 9% and 13% rubber, containing at least 5% of its weight of resin; substantially 15% of factice; substantially 18% heavy spar; and substantially 7% mineral oil and over 13% of lithopone. 85

In testimony whereof, we have signed our names to this specification.

JOSEF TALALAY.  
WILHELM HOLZBERG.

90

100

105

110

115

120

125

130